

## UNITED STATES PATENT OFFICE

2,068,635

## ENGINE FUEL

Carl F. Prutton, Cleveland, Ohio, assignor, by  
mesne assignments, to The Lubri-Zol Develop-  
ment Corporation, Cleveland, Ohio, a corpora-  
tion of Delaware

No Drawing. Application December 29, 1932,  
Serial No. 649,329

12 Claims. (Cl. 44—9)

This invention relates, as indicated, to engine fuel and more particularly such fuel as is consumed by internal combustion engines, and which has added thereto certain compositions 5 which increase the efficiency of operation of the engine as well as insure a minimum of wear of the parts of such engine.

It has for some time past been realized that the lubrication of the upper parts of an engine, 10 i. e., the piston, piston rings, valves, etc., can be improved by the addition to the engine fuel of a suitable lubricating composition, and for such purpose pure hydrocarbon oils have been employed as well as other mixtures and suspensions 15 which are dissolved in the fuel and admitted to the combustion chamber of the engine through the carburetor and manifold. Plain hydrocarbon oils have a tendency to produce undesirable amounts of carbon deposit and are generally not 20 sufficiently stable, at the temperatures encountered in the combustion chamber, so that the use of plain hydrocarbon oils for the above defined purpose has never gone into extensive commercial usage.

25 It is among the objects of this invention to provide an engine fuel suitable for consumption by internal combustion engines, and which has mixed therewith a composition which will not only reduce friction between the working parts 30 of the engine but which is sufficiently stable so as not to produce carbon deposits and further is effective to soften and loosen carbon deposits which have been formed or which are formed by the combustion of the fuel.

35 For the purpose of lubricating or reducing the friction between the relatively moving parts of the engine such as the piston and cylinder, piston rings, valves, etc., this invention contemplates the addition to any suitable fuel, adapted for internal combustion engines, of a lubricating composition comprising a major proportion of a suitable oil base and a minor proportion of a halogenated or more specifically chlorinated carbon ring compound. As specific examples of the 40 halogenated or more specifically chlorinated carbon ring compounds which may be employed as compositions in combination with a suitable oil for the purpose of reducing friction are halogenated or chlorinated compounds of benzene, naphthalene, diphenyl, substituted benzene, substituted naphthalene and substituted diphenyl. Specific examples of the above enumerated compounds are mono-chlor-benzene, di-chlor-benzene, notably the ortho compound, chlor-naphthalenes, chlor-diphenyls, as well as chlorinated 45

homologs of the above, such as toluene, alpha methyl naphthalene and phenyl toluene.

In addition to the above enumerated class of compounds, halogenated oxygen bearing carbon ring compounds, such as compounds of the class 5 including halogenated oxygen bearing compounds of substituted benzene, substituted naphthalene and substituted diphenyl, may be employed. As specific examples of this last named group of oxygen containing compounds, the following will be found to produce satisfactory results, viz., as examples of chlorinated oxygen containing substituted benzene compounds, chlorinated phenols, cresols, diphenyl ether, methyl salicylate; as examples of halogenated 15 substituted diphenyl, chlorinated para-phenyl phenol and chlorinated dixenyl ether; and as an example of chlorinated substituted naphthalenes, chlorinated naphthols.

In addition to the above enumerated compounds, halogenated aromatic ethers, phenols, acids and esters, and aldehydes, have been found to produce desirable results.

The above enumerated halogenated oxygen-bearing compounds hydrolyze somewhat more 20 readily than the corresponding hydrocarbon compounds and accordingly the selection and use of such oxygen-containing compounds must be with greater care on account of the possibility 25 of their effecting corrosion at least to a minor 30 degree. It will be observed that all of the above enumerated halogenated oxygen-bearing carbon ring compounds consist entirely of carbon hydrogen, oxygen and halogen.

35 It will also be noted that all of the above enumerated examples of halogenated carbon ring compounds are of the aryl type, i. e., compounds containing benzenoid ring structures and are also of the type in which the halogen is directly attached to an atom which is a part of such ring 40 structure.

The amount of halogenated compound added to the oil base may vary somewhat according to the particular compound added as well as the 45 particular usage in view, and may range up to, for instance, about 20%. Mixture occurs readily and at ordinary temperatures.

The optimum amount of halogenated compound added will depend upon the halogen content of the compound, its physical character, especially its effect on the viscosity of the oil to which it is added, and also upon the particular characteristics of the use for which the composition is intended. When the lubricant is combined 50

with the usual gasoline for internal combustion engines, the lubricating composition will preferably contain from 2 to 10 per cent. of halogenated compounds.

- 5 As previously indicated, the lubricant having combined therewith compositions such as have been above enumerated may be mixed with or dissolved in any suitable type of fuel for internal combustion engines so that after vaporization 10 and combustion in the cylinders of the engines consuming such fuel, there will be a remainder on the walls of such cylinder and adjacent working parts, such as valves, of the lubricating composition.
- 15 For proper results, a lubricant compounded from a relatively heavier hydrocarbon lubricant in the previously indicated manner should be added to the usually lighter hydrocarbon engine fuel in quantities varying from .05 per cent to 20 1.50 per cent by volume. The amount of lubricant added to the fuel for optimum results will be found to be in the vicinity of .30 per cent, i. e., .15 per cent to .60 per cent. It will be noted that the actual percentage of halogenated compounds 25 of the previously enumerated classes, which will be present in the fuel mixture, will be considerably less than the percentages just given due to the fact that the lubricating composition added to the fuel itself contains only a minor proportion 30 of these compounds, as previously explained.
- Fuel compositions of the character described 35 are capable of providing superior valve lubrication and exhibit marked penetration while at the same time the advantage of low volatile oil body is had. A further particular advantage lies in the tendency of such a compounded fuel to keep down carbon formation and to soften and loosen any carbon which may form. The cold test of 40 the lubricating composition added to the fuel is very low, thus rendering the same particularly useful in engines in cold weather or in aviation.
- Other modes of applying the principle of my 45 invention may be employed instead of the one explained, change being made as regards the composition herein disclosed, provided the ingredients stated by any of the following claims or the equivalent of such stated ingredients be employed.
- I therefore particularly point out and distinctly 50 claim as my invention:
- 50 1. The method of forming a liquid motor fuel which comprises adding thereto a small quantity of a lubricating composition containing high boiling hydrocarbons in amounts greater than any normally present in the fuel, said lubricating 55 composition likewise containing an effective amount less than 20% of a halogenated carbon ring compound of the type in which substantially all of the halogen present is attached to the ring structure.
- 60 2. An internal combustion engine fuel comprising a liquid hydrocarbon fuel having dissolved therein a small quantity of a lubricating composition consisting principally of high boiling hydrocarbons so that the content in the fuel of such 65 constituents is increased, said lubricating composition likewise containing an effective amount less than 20% of a halogenated carbon ring compound of the type in which substantially all of the halogen present is attached to the ring structure.
- 70 3. An internal combustion engine fuel comprising a liquid motor fuel of the type boiling within the gasoline range and a composition dissolved therein which consists principally of a suitable relatively heavier hydrocarbon lubricating oil, and an effective amount less than 20% 75

based on said lubricating oil, of a halogenated carbon ring compound of the type in which substantially all of the halogen is attached to the ring structure.

4. An internal combustion engine fuel comprising a hydrocarbon fuel and a composition dissolved therein which consists principally of a suitable hydrocarbon lubricating oil, and an effective amount less than 20% based on said lubricating oil, of a halogenated, oxygen-bearing 10 carbon ring compound consisting entirely of carbon, hydrogen oxygen and halogen and being of the type in which substantially all of the halogen is attached to the ring structure. 15

5. An internal combustion engine fuel comprising a liquid motor fuel of the type boiling within the gasoline range and a composition dissolved therein which consists principally of a suitable relatively heavier hydrocarbon lubricating oil, and from about 2% to 10% based on 20 said lubricating oil of a halogenated carbon ring compound of the type in which substantially all of the halogen is attached to the ring structure. 25

6. An internal combustion engine fuel comprising a liquid motor fuel of the type boiling within the gasoline range and from about 0.05% to 1.5% by volume of a composition dissolved 30 therein which consists principally of a suitable relatively heavier hydrocarbon lubricating oil, and an effective amount less than 20% based on said lubricating oil of a stable, non-corrosive halogenated carbon ring compound of the type in which substantially all of the halogen is attached to the ring structure. 35

7. An internal combustion engine fuel comprising a liquid motor fuel of the type boiling within the gasoline range and from about 0.15% to 0.60% by volume of a composition dissolved therein which consists principally of a suitable relatively heavier hydrocarbon lubricating oil, 40 and an effective amount from about 2% to about 10% based on said lubricating oil of a chlorinated carbon ring compound of the type in which substantially all of the chlorine is attached to the ring structure. 45

8. An internal combustion engine fuel comprising a liquid motor fuel of the type boiling within the gasoline range and a composition dissolved therein which consists principally of a suitable relatively heavier hydrocarbon lubricating oil, and an effective amount less than 20% based on said lubricating oil of a halogenated carbon ring compound of the class consisting of halogenated homologs of aromatic hydrocarbons of the type represented by benzene, naphthalene 55 and diphenyl, which compounds are of the type in which substantially all of the halogen is attached to the ring structure.

9. An internal combustion engine fuel comprising a liquid motor fuel of the type boiling within the gasoline range and a composition dissolved therein which consists principally of a suitable relatively heavier hydrocarbon lubricating oil, and an effective amount less than 20% based on said lubricating oil of a halogenated 60 carbon ring compound of the class consisting of halogen and oxygen-bearing derivatives of aromatic compounds of the type represented by benzene, naphthalene and diphenyl and consisting entirely of carbon, hydrogen, oxygen and halogen with substantially all of the halogen attached to the ring structure. 65

10. An internal combustion engine fuel comprising a liquid motor fuel and a composition dissolved therein which consists principally of a 70

suitable hydrocarbon lubricating oil, and an effective amount less than 20% of o-dichlorbenzene.

11. An internal combustion engine fuel comprising a liquid motor fuel and a composition dissolved therein which consists principally of a suitable hydrocarbon lubricating oil, and an ef-

fective amount less than 20% of halogenated diphenyl ether.

12. An internal combustion engine fuel in accordance with claim 2, in which the halogenated carbon ring compound is chlorinated dixenyl 5 ether.

CARL F. PRUTTON.